

Patented Apr. 27, 1926.

1,582,705

## UNITED STATES PATENT OFFICE.

ARNOLD M. TAYLOR AND FRANK A. BUOTE, OF STAMFORD, CONNECTICUT, ASSIGNORS  
TO ATLAS POWDER COMPANY, OF WILMINGTON, DELAWARE, A CORPORATION OF  
DELAWARE.

## FLOOR PUTTY HAVING A NITROCELLULOSE OIL BASE.

No Drawing.

Application filed March 11, 1925. Serial No. 14,834.

*To all whom it may concern:*

Be it known that ARNOLD M. TAYLOR and FRANK A. BUOTE, citizens of the United States, residing at Stamford, in the county 5 of Fairfield and State of Connecticut, have invented certain new and useful Improvements in a Floor Putty Having a Nitrocellulose Oil Base, of which the following is a specification.

10 This invention relates particularly to floor putties having a nitrocellulose-oil base, the object of the invention being to provide a putty which is especially adapted for use under pyroxylin finishing compositions, al- 15 though it may function under materials other than pyroxylin finishing compositions with equal facility.

It is a recognized fact that in the art of 20 floor finishing, when a pyroxylin finishing composition is applied directly over an ordinary commercial putty in which the liquid vehicle is not thoroughly dry, or not absorbed to a large extent by the inert filling material contained in the putty, the solvents 25 in the pyroxylin material attack the liquid vehicle, causing a marked tackiness to develop accompanied in most cases by a bleaching action of the tinted putty. This is similar to the bleaching action which 30 takes place when a pyroxylin finishing composition is applied directly over certain tinted wood fillers which have not dried sufficiently. A putty which has incorporated in it certain coloring materials is 35 usually deprived of its color by the effect of a pyroxylin composition over it. We attribute this effect to the washing away of the tinting materials which leaves the predominating pigment exposed and this pigment is usually white or transparent.

When a pyroxylin finishing composition is applied over a putty containing a nitrocellulose-oil base, the pyroxylin solvents present in such a composition do not exhibit 45 the effect of washing away the tinting colors as described above, but the pyroxylin finishing composition penetrates the nitrocellulose-oil putty to such an extent that it combines firmly with it and there is no tendency

for the oil in the nitrocellulose-oil putty to 50 come to the surface and cause tackiness. There is apparently no deleterious effect exhibited on the tinting colors in a nitrocellulose-oil putty when a pyroxylin finishing composition is applied over it but instead 55 the tinting colors seem to be well protected by the nitrocellulose-oil putty, because the pyroxylin finishing composition dissolves the nitrocellulose-oil putty to a certain extent and upon drying envelops the pigments, 60 thus preventing their being washed away by the pyroxylin solvents.

The nature of an ordinary commercial 65 putty is such that when it is used for filling the cracks of a floor, for example, a considerable period of time must elapse before it is sufficiently dry to proceed with the finishing coats. Under this condition 70 there is always a tendency to apply the finishing coats before the putty is thoroughly dry which results in decreased wearing qualities of the final finish because the putty is soft and affords an infirm foundation for the finishing materials.

The putty to which this invention relates 75 dries much faster than an ordinary commercial floor putty and therefore affords a firm foundation over which to apply pyroxylin finishing compositions. In a finishing operation where considerable putty is 80 used, the advantages of a putty of this nature can be readily appreciated as regards the saving of time and improvement of wearing qualities of the final finish.

The formula given below is representative 85 of a floor putty containing a nitrocellulose-oil base:

|                | Parts. |
|----------------|--------|
| Butyl acetate  | 48     |
| Vegetable oil  | 36     |
| Nitrocellulose | 10     |
| Clay           | 100    |

While we prefer to use clay, English 95 china clay for example, other earth pigments may be employed in lieu thereof. We combine any suitable tinting materials with the above described base to secure the

desired color of the finished product. While we contemplate using any suitable vegetable oil, we may mention linseed oil as an example of a suitable oil for our purpose. To the best of our knowledge we are the first to provide a nitrocellulose putty for use under pyroxylin coatings. Therefor it is to be understood that by the term "putty" as used in the appended claims, is meant 10 a product sufficiently stiff and tenacious to permit of its use as a crack filler under pyroxylin coatings, without danger of its "pulling out" of such cracks under the action of a brush, and that by the term "of 15 the character described" is meant a putty particularly intended and adapted for use under pyroxylin coatings.

We wish it to be understood that many changes may be made in our invention without departing from the spirit thereof, and although a putty made according to the specifications above given, is especially suited for use under pyroxylin compositions, we do not wish to limit its use to this purpose alone.

We claim the following:

1. A putty of the character described comprising the following ingredients, com-

bined in substantially the proportions stated:

|                           | Parts. |
|---------------------------|--------|
| A nitrocellulose solution | 58     |
| A vegetable oil           | 36     |
| Clay                      | 100    |

2. A putty of the character described comprising a nitrocellulose solution, a vegetable oil and an earth pigment, combined in such proportions that the combined amount of the nitrocellulose solution and vegetable oil is substantially equal to the amount of the earth pigment.

3. A putty of the character described comprising the following ingredients combined in substantially the proportions stated, viz:

|                | Parts. |
|----------------|--------|
| Butyl acetate  | 48     |
| Vegetable oil  | 36     |
| Nitrocellulose | 10     |
| Clay           | 100    |

In testimony whereof they affix their signatures.

ARNOLD M. TAYLOR.  
FRANK A. BUOTE.